

Jan. 31, 1928.

P. SCHWARZKOPF

1,657,553

ANODE AND METHOD OF MAKING THE SAME

Filed June 15, 1922



Inventor:  
Paul Schwarzkopf  
By Hilmer Owen  
His Attorney

## UNITED STATES PATENT OFFICE.

PAUL SCHWARZKOPF, OF CHARLOTTENBURG, GERMANY, ASSIGNOR OF ONE-HALF TO  
DEUTSCHE GLÜHFADENFABRIK, RICHARD KURTZ & DR. ING. PAUL SCHWARZ-  
KOPF, G. M. B. H., OF BERLIN, GERMANY.

## ANODE AND METHOD OF MAKING THE SAME.

Application filed June 15, 1922; Serial No. 568,521, and in Germany June 21, 1921.

My invention relates to an anode for Röntgen apparatus and a process of making the same. The invention consists in the structure of the anode and the method of producing it, which will appear in detail as the description proceeds.

In the accompanying drawings, Figure 1 shows an anode such as has been hitherto used; Figures 2 and 3 are sections on the lines A—B and C—D, respectively, on Fig. 1; Figs. 4 and 5 are face and side views, respectively, of one form of my improved anode; Fig. 6 shows a side view of a modified form of the same; Fig. 7 is a diagrammatic view indicating the operation of the anode shown in Fig. 1; Figs. 8 and 8<sup>a</sup> are face and side views, respectively, indicating the arrangement of the fibers of the metal in my improved anode; Fig. 9 is a side view of a further modified form of my improved anode.

Anodes for Röntgen tubes have been made of tungsten and similar metals. In working tungsten, molybdenum, and similar difficultly fusible metals, bars are first formed by sintering compressed powdered material. These bars are usually sintered by passing an electric current through them, preferably while surrounded by neutral gases. It is difficult to form bars of any considerable size in this manner. A bar having a thickness of 15 or 20 millimeters and a length of 15 or 20 centimeters requires a current of thousands of amperes. For this reason the size of such bars is very limited. The material is so refractory that bars of even this size cannot be formed practicably by fusion and casting.

Bars formed in this manner have been rolled lengthwise to form strips or plates for various purposes. These strips or plates have not been more than 30 millimeters in width, as the longitudinal rolling of the bars does not greatly increase their width. Furthermore, when such bars are rolled the edges of the strip do not have the same structure as the central portion of the strip, but are likely to be cracked and inferior.

In making such an anode as shown in Fig. 1, a sintered bar has one end drawn out, as shown at s in Fig. 1, while the other end h remains in substantially the original con-

dition. If it is worked at all it will be stretched lengthwise, but any such working must be slight in order to retain the desired extent of surface on the receiving end f.

In forming my improved anode, a sintered bar may be used having a less diameter than the bar used to form the anode shown in Fig. 1. The entire bar is preferably lengthened by mechanical treatment, as by hammering or rolling to lengthen it to some extent. This preliminary lengthening is not absolutely necessary, but is preferable in order to compact the material and give it the desired strength for subsequent treatment.

After the lengthening, the end which is to form the anode is broadened by mechanical treatment, as by hammering or rolling, until it attains the desired form. The anode may be used in the shape shown in Figs. 4 and 5 or may be given a V-shape, such as shown in Fig. 6. This V-shape is preferred. The plate may be bent from the shape shown at g in Fig. 5 to the shape shown at h in Fig. 6 while the metal is hot, or it may be formed directly in the shape shown in Fig. 6 by rolling it with suitably shaped rollers. If desired, the plate may be made long enough so that it can be bent as shown in Fig. 9, the side i presenting the receiving surface, while the bent front end j will constitute a cooling rib; in any case where the V-shape is given the plate, any portion of the plate which is at an angle to the receiving surface will act as a cooling rib. The portion j of the plate may be bent at right angles, as shown in full lines in Fig. 9, or it may be bent up to the position shown in dotted lines in that figure.

The advantages of my improved anode and the manner of making it may be briefly stated as follows:

In the first place a bar of less diameter may be used, thereby saving metal. The smaller bar can be made with much less difficulty than the larger bar for reasons indicated above. In the next place, the anode will have much more cooling surface in proportion to the amount of metal contained. Furthermore, the structure of the plate is such as to make it more durable. In the form of anode shown in Fig. 7, the portion h is either porous and entirely untreated or

it has such treatment as will tend to create fibers running longitudinally of the anode, as shown at *a*. In my improved anode, the receiving surface has been given mechanical treatment both lengthwise and transversely, so that the material is comparatively dense. Furthermore, the transverse working takes place after the longitudinal working and is considerably more extensive, so that the fibers extend transversely, as indicated at *a* in Figs. 8 and 8<sup>a</sup>. In all instances the fibers in the portion *s* will run longitudinally of the holder. This is desirable in the holder, but in the receiving surface of the anode itself, it is undesirable. When the rays or electrons strike the anode in the direction indicated by *p* in Figs. 7, 8 and 8<sup>a</sup>, there is a tendency to pit a porous surface, such as presented by the anode shown in Fig. 7, and this tendency is not at all lessened by fibers running longitudinally of the anode or approximately perpendicular to the receiving surface; but the comparatively compact surface of an anode such as shown in Figs. 8 and 8<sup>a</sup>, is further strengthened by the transverse fibers indicated in those figures and, therefore, resists pitting to a much greater extent.

While I have disclosed a specific embodiment of my invention, it will be obvious that various departures from the disclosure may

be made within the scope of the appended claims without departing from the spirit of my invention.

What I claim is:

1. An anode for a Röntgen tube comprising a receiving surface of fibrous metal having its fibers transverse the direction of the current.

2. An anode for a Röntgen tube comprising a receiving plate of fibrous metal having its fibers transverse the direction of the current and having an integral supporting bar.

3. An anode for a Röntgen tube comprising a receiving plate of fibrous metal having its fibers transverse the direction of the current and having an integral supporting bar of fibrous metal, the fibers in the said bar running parallel with the current.

4. In a Röntgen ray device, a plate-shaped anode, the crystals of which extend in a plane enclosing an angle with the direction of travel of electrons.

5. In a Röntgen ray device, an anode in the form of a flat plate having a rod at one end, the crystals of said plate extending in the plane thereof, and the cross section of said plate being at an angle to the cross section of the rod.

DR. PAUL SCHWARZKOPF.